

April 24, 1928.

1,667,146

J. L. DRAKE

SHEET OF GLASS AND PROCESS OF PRODUCING THE SAME

Filed March 27, 1926



Inventor

John L. Drake.

Frank Frank.

Attorney

Patented Apr. 24, 1928.

1,667,146

# UNITED STATES PATENT OFFICE.

JOHN L. DRAKE, OF TOLEDO, OHIO, ASSIGNOR TO THE LIBBEY-OWENS SHEET GLASS COMPANY, OF TOLEDO, OHIO, A CORPORATION OF OHIO.

## SHEET OF GLASS AND PROCESS OF PRODUCING THE SAME.

Application filed March 27, 1926. Serial No. 97,900.

The present invention relates to sheet glass, and to an improved process for producing the same.

An important object of the invention is 5 to provide an improved process adapted for the production of a new article of manufacture, namely, a sheet of ground and fire-polished glass.

Another object of the invention is to provide a process wherein a sheet of glass may 10 be ground and then fire-polished.

A further object of the invention is to provide a process wherein a sheet of glass may be formed, after which the surfaces 15 thereof may be ground, the ground sheet being reheated and then subjected to a flame to fire-polish the ground surfaces, the sheet then being slowly reduced to room temperatures.

20 Other objects and advantages of the invention will become apparent during the following description.

In the drawings wherein like numerals are employed to designate like parts 25 throughout the same,

Fig. 1 is a diagrammatic view illustrating a sheet being ground and reheated,

30 Fig. 2 is a sectional view showing diagrammatically the end of the reheating means, the fire-polishing of the sheet, and the starting of the cooling operation, and

Fig. 3 is a diagrammatic view illustrating the exit of the sheet after it has been cooled.

35 The present invention relates particularly to the production of so-called "plate glass", wherein a glass blank is ground and polished in a manner that the surfaces of the sheet are substantially flat and parallel, thus reducing to a minimum distortion of vision 40 therethrough. It has been customary heretofore in the production of sheet glass to grind a blank and then polish the same by a rubbing action of a suitable polishing compound such as rouge applied by means of a 45 felt pad.

In the present invention the grinding is 50 accomplished by any of the well known methods now in vogue, while the polishing is accomplished by means of a flame or fire, giving the sheet what is known as a fire-polish. By grinding the sheet prior to its polishing, in accordance with the present invention, all surface defects are removed so 55 that a ground blank is produced having

flat surfaces and a sheet of uniform thickness.

In the drawings the numeral 5 designates diagrammatically a sheet glass grinding machine. By means of the grinding head 6 the 60 sheet 7 may be ground on both of its surfaces by grinding first one side and then turning the sheet over and grinding the second side.

After the sheet has been ground on both 65 sides it may then be passed through a reheat- 70 ing chamber 8. The chamber 8 preferably includes a plurality of rotatable rolls 9, adapted to support the sheets 7 in their passage through said chamber. Suitable heat- 75 ing means 10 may be used to gradually elevate the temperature of the glass sheets. The sheet, after it has become suitably heated, may then pass upon a moving table 11, where it is subjected to the action of a 80 flame 12 of sufficient intensity to produce what is known in the art as a fire-polish upon the ground surface of the sheet 7. The flame is preferably what may be called a "sharp" flame adapted to "lick" the surface 85 of the sheet so that it will polish the surface of the sheet of glass with which it contacts without destroying the uniformity of thickness of the sheet. By using this type of flame the very surface of the sheet can be melted so to speak, without causing a breakdown of the body of said sheet. Of course, the melting referred to is sufficient to cause fire polishing of the ground surfaces. One or a plurality of flames 12 may 90 be applied to the sheet as desired. After one side of the sheet has been fire-polished, it may be reversed as indicated at 13, and the second side of the sheet may be fire-polished as by means of the flame 14. The table 95 11, supported upon the means 15, may be housed by means of a cover 16, and any suitable turnover device may be used to turn the sheet 7 after one side has been polished. After the second side of the sheet has been 100 polished, it is then passed through a cool- 105 ing chamber 17. This chamber preferably includes rotatable supporting means 18 and heating means 19, whereby the sheet is gradually reduced to room temperatures. After the sheet has been cooled, it is passed out upon a table 20, from where it may be removed and examined as desired.

Of course, it is to be understood that the sheet 7 is annealed prior to the grinding op- 110

eration. In other words, the sheet or blank 7 is produced in the customary manner including the ordinary annealing operation. The cooling chamber 17 is used to bring the heated sheet 7 to room temperatures after it has been fire-polished. It is not absolutely necessary to reheat the sheet 7 before it is fire-polished, but the danger of breakage is considerably lessened if it is reheated.

10. It is well known in the art that a fire-polish or a fire finish has more luster than the finish sometimes produced by a rubbing action. A piece of plate glass produced by the above described apparatus can be made much more cheaply than with the rubbing process.

Of course both surfaces of the sheet may be fire-polished simultaneously by moving the same on spaced rolls and applying a flame on both of the surfaces by arranging them above and below the sheet.

20. It is to be understood that the form of the invention herewith shown and described is to be taken as the preferred embodiment of 25 the same, and that various changes in the shape, size and arrangement of parts may be resorted to without departing from the spirit of the invention or the scope of the subjoined claims.

30. I claim:

1. The process of producing a transparent sheet of glass, consisting in grinding a sheet of glass, and then fire-polishing the same.

2. The process of producing plate glass, 35 consisting in grinding both sides of a sheet of glass, and then fire-polishing the same.

3. The process of finishing sheet glass, consisting in grinding a sheet of glass, heating the same, and then polishing said sheet.

40. 4. The process of finishing sheet glass, consisting in grinding a sheet of glass, heating the same, and then fire-polishing said sheet.

45. 5. The process of finishing a sheet of glass, consisting in grinding the sheet, then

passing it through a heated chamber, and then polishing the same.

6. The process of finishing a sheet of glass, consisting in grinding the sheet, then passing it through a heated chamber, and 50 then fire-polishing the same.

7. The process of finishing a sheet of glass, consisting in grinding the sheet, passing the same through a heated chamber, polishing the same, and then cooling said sheet. 55

8. The process of finishing a sheet of glass, consisting in grinding the sheet, then passing the same through a heated chamber, fire-polishing the same, and then cooling said sheet. 60

9. The process of producing polished sheet glass, consisting in grinding the surfaces of a sheet of glass, gradually elevating the temperature of said sheet, then subjecting the heated ground surfaces to the action 65 of a flame to fire-polish the same.

10. The process of producing polished sheet glass, consisting in grinding the surfaces of a sheet of glass, gradually elevating the temperature of said sheet, subjecting the 70 heated ground surfaces to the action of a flame to fire-polish the same, and then cooling said sheet.

11. The process of producing polished sheet glass, consisting in grinding both surfaces of a sheet of glass, passing the ground sheet through a heating chamber, fire-polishing one side of the sheet, then turning the sheet over and fire-polishing the second side, and then cooling said sheet. 75

12. As a new article of manufacture, a sheet of glass which has been ground, reheated and fire-polished.

13. As a new article of manufacture, a sheet of glass which has been ground and 85 fire-polished.

Signed at Toledo, in the county of Lucas and State of Ohio, this 25th day of March, 1926.

JOHN L. DRAKE.